

Patented Apr. 27, 1926.

1,582,420

# UNITED STATES PATENT OFFICE.

YASUJURO NIKAIDO, OF ROSSFORD, OHIO.

## MOTOR FUEL.

No Drawing.

Application filed July 9, 1925. Serial No. 42,587.

To all whom it may concern:

Be it known that YASUJURO NIKAIDO, citizen of Japan, residing at Rossford, in the county of Wood and State of Ohio, has invented certain new and useful Improvements in Motor Fuels, of which the following is a specification.

My invention relates to motor fuels. More specifically, it relates to the production of an improved hydrocarbon motor fuel possessing among other properties that of accelerating ignition.

I have discovered that a highly advantageous water fuel may be formed by mixing a hydrocarbon or a hydrocarbon derivative with a small proportion of an ether adapted to accelerate ignition of the fuel and which does not require a blending agent to incorporate it with the other constituents of the fuel.

Mixtures of hydrocarbons and mono-alkyl ethers such as methyl and ethyl ether are well known. The addition of ethers of this type does aid in the combustion of hydrocarbons such as gasoline but they have the disadvantage of easily separating and evaporating from the gasoline and therefore in order to minimize this tendency, it is necessary to use a blending agent for example, benzol. The dialkyl ethers, preferably those containing low alkoxy radicals and especially formal



do not require any blending agent and in addition confer other beneficial qualities on the fuel as will be more fully hereinafter pointed out.

Examples of dialkyl ethers which may be added to hydrocarbons are:

Formal or methylal,



diethyl formal or methylene diethyl ether



acetal,



dimethyl acetal,



55

Glycol compounds, for example, the glycol ethers, such as glycol methylene acetal



60

and glycol diethyl ether



which is an isomer of acetal are also suitable. 65 The glycol ethers containing two alkoxy radicals for example,  $\text{OC}_2\text{H}_5$ , may be included under the term dialkyl ethers and it is desired that this term as used in the specification and claims be given this significance.

Mixtures of hydrocarbon compounds with my ignition accelerator have been tried out in practice and found to be very advantageous. In general, in making up the motor fuel for use, four fluid ounces of the ignition accelerator are mixed with ten gallons of the hydrocarbon, for example, gasoline. This proportion makes approximately three parts by volume of the ignition accelerator to one thousand parts by volume of gasoline. Other mixtures have been tried containing from one to six parts of the ignition accelerator to one thousand parts of the hydrocarbon, such as gasoline. The most satisfactory results, however, have been obtained by having three parts of the ignition accelerator present in one thousand parts of the hydrocarbon.

The following experiments were carried out with the mixtures stated:

A Dodge sedan, 1918 model was tested in cold weather using straight gasoline. The following results were obtained:

1. It was noted that it started with difficulty.

2. The choker had to be pulled out all the time while running.

3. The machine could not be throttled down to less than six to seven miles per hour without jolting.

4. One of two cylinders were missing exploding.

Using the same gasoline with three parts

of formal per thousand parts of gasoline the following results were noted:

1. That the machine started readily even though the weather was cold.

5 2. The choker could be left pushed in as far as it would go while the machine was running.

10 3. A large amount of old soot or carbon was blown out through the exhaust, this signifying that the new fuel had the effect of cleaning the fouled engine cylinders with carbon.

15 4. After driving the machine for a mile, all the cylinders were "hitting". This was undoubtedly due to a cleaner engine.

5. The machine could be slowed down until the speedometer indicated a speed of less than one mile without the slightest jolting.

20 My improved fuel was tested in a very old Willys-Knight coupé. The ignition in this machine was performed by a magneto as there was no battery.

Using straight gasoline is was noted that:

25 1. The machine started with difficulty in cold weather.

2. The choker had to be pulled out all the time the engine was running. If the choker was pushed in, the engine back-fired badly.

30 3. The machine could not be slowed down to less than ten miles per hour without badly jolting and finally stalling.

Using my improved fuel with three parts of formal per thousand parts of gasoline, the following results were noted:

35 1. The starting was improved to a remarkable degree.

2. The choker could be pushed in as far as it would go during the entire time the engine was running even though the weather was cold and no back-firing occurred. This signifies that the ignition occurred with a thinner mixture of gasoline and air when the ignition accelerator is present in the mixture than when it is not.

45 3. The machine could be slowed down so that it just crept along without jolting and stalling. This indicates that the ignition occurs with a very slight spark as the magneto gives only a very small spark when the car is running slowly.

Experiments carried out in cold weather on a Ford sedan, 1924 model gave the following results:

55 1. When using straight gasoline the engine could only be started with great difficulty.

2. The engine could not be throttled down to less than ten miles per hour without badly jolting and stalling.

60 3. Using gasoline containing three parts of formal per thousand parts of the gasoline, it is noted that,

1. The starting is improved remarkably and

2. The engine could be throttled down to less than five miles without any jolting or stalling.

Experiments were carried out using my improved fuel on a Lincoln touring car, 1925 model. These experiments did not include starting the engine with the improved fuel but the fuel was tried out after the engine had been started. Using straight gasoline it was noted that:

1. The fume from the exhaust was so strong and disagreeable that it made persons unaccustomed thereto ill.

2. The machine began to jolt when it was slowed down to less than five miles per hour.

Using gasoline containing three parts of formal per thousand parts of gasoline, the following were noted:

1. The fume from the exhaust lost its usual strong disagreeable odor. A person could hold his face in front of the muffler without ill effects.

2. The machine could be slowed down to about 2.5 miles per hour without jolting. The machine crept along quietly without any jolting.

3. The use of the improved fuel resulted in an increased mileage of about 10%.

By using equal quantities of the straight gasoline and the improved fuel a 10% increase of mileage results when using the latter.

Other members of the dialkyl ether series were tested using the same proportions of the ignition accelerators to gasoline as mentioned above.

Specific examples of improved fuel are as follows:

|                                                                                                      |          |     |
|------------------------------------------------------------------------------------------------------|----------|-----|
| 1. Gasoline .....                                                                                    | 10 gals. | 105 |
| Formal or methylal, sometimes called methylene dimethyl ether, $\text{CH}_2\text{OCH}_2\text{OCH}_3$ | 4 oz.    |     |
| 2. Gasoline .....                                                                                    | 10 gals. | 110 |
| Diethyl formal, or methylene diethyl ether, $\text{CH}_2\text{OC}_2\text{H}_5\text{OC}_2\text{H}_5$  | 4 oz.    |     |
| 3. Gasoline .....                                                                                    | 10 gals. | 115 |
| Acetal, ethyldiene diethyl ether, $\text{CH}_2\text{CH}(\text{OC}_2\text{H}_5)_2$                    | 4 oz.    |     |
| 4. Gasoline .....                                                                                    | 10 gals. | 120 |
| Dimethyl acetal, $\text{CH}_3\text{CH}(\text{OCH}_3)_2$                                              | 4 oz.    |     |

Of the above series, the best results are obtained when formal, methylene dimethyl ether, is used. The other members of the se-

ries give satisfactory results but the preferred ignition accelerator to be used in my improved fuel is formal.

The glycol compounds can also be used, especially the glycol ethers, for example, glycol methylene acetal,



10 and the glycol diethyl ether,



15 The halogen substituted dialkyl ethers including the halogen substituted glycols may in some cases be substituted for the above set forth compound.

20 The dialkyl ethers are admirably adapted to be blended with gasoline since they have relatively low boiling points. For example, formal boils at 42° C. Its specific gravity is .855. The dialkyl ethers may be obtained by mixing aldehyde and alcohol in the presence of a catalyst such as hydrochloric acid or by heating the mixture to 100° C. without a catalyst. The dialkyl ethers dissolve in and mix with water in all proportions. When heated with water and sulfuric acid 25 the members of the series break down into aldehydes and alcohols.

30 My experiments have indicated that the beneficial results flowing from the use of the dialkyl ethers, especially formal, are much more noticeable in the cheaper grade of cars than with the expensive cars such as the Packard or the Lincoln which are equipped with more perfect combustion mechanism. My experiments have also indicated that the 35 beneficial results flowing from the use of the dialkyl ethers, especially formal, are much more noticeable when using ordinary gasoline than when high test gasoline is used.

40 Summarizing, the following advantages 45 are obtained by the use of the compounds set forth:

1. The starting of the car especially in cold weather is greatly improved.  
50 2. These compounds prevent or at least greatly lessen the knocking.  
3. The car runs smoothly without jolting.  
4. The improved fuel cleans the old soot or carbon from the fouled engine cylinders.  
55 5. The deposition of carbon is totally prevented or at least greatly minimized.  
6. Increased mileage is obtained.

7. A car may be driven more slowly without jolting when using the improved fuel 60 than when using straight gasoline.

8. No poisonous effects are obtained when using compounds of the character set forth as the combustion products of the same are substantially harmless under ordinary condi-

tions, for example, the combustion products 65 of formal are carbon dioxide and water.

9. These compounds remain mixed with gasoline indefinitely without any blending agents.

10. The ignition of the fuel mixture containing the dialkyl ethers takes place with a 70 very slight spark.

11. The usual disagreeable sickening odor of the exhaust draft is totally removed or 75 at least greatly minimized.

It is obvious that compounds of the character set forth may be added to hydrocarbons in general. While in the examples given only gasoline has been used, the gasoline may be substituted by a mixture of heavy hydrocarbon and gasoline. It is also obvious that a substantial proportion of benzol may be added to the hydrocarbon where this is desirable. The alcohol fuels are also improved by the use of the compounds set forth. It is not desired that my invention be limited to any specific type of fuel but protection is desired on the use of the compounds set forth in connection with the use of fuel hydrocarbon or fuel hydrocarbon derivatives under which term alcohol is included.

It is to be noted that in all the examples set forth the percentage of ignition accelerator is relatively small. Usually the latter is less than one half per cent although it may rise to one per cent or even somewhat greater. In my fuel compounds of the character set forth especially formal and compounds of this series are used in small quantities as a catalyst or accelerator of ignition and it is for this reason, that it is not necessary to use large quantities of these compounds.

The term, "dialkyl ether" as used in the claims excludes "mono-alkyl ethers" such as "diethyl ether". A dialkyl ether contains two alkoxy radicals.

I claim:—

1. A motor fuel containing a hydrocarbon and a small proportion of a dialkyl ether having a boiling point below 104° C. adapted to accelerate ignition.

2. A motor fuel containing a light hydrocarbon and a small proportion of a dialkyl ether having a boiling point below 104° C. adapted to accelerate ignition.

3. A motor fuel containing gasoline and a small proportion of a dialkyl ether having a boiling point below 104° C. adapted to accelerate ignition.

4. A motor fuel containing a hydrocarbon and formal adapted to accelerate ignition.

5. A motor fuel containing a light hydrocarbon and formal adapted to accelerate ignition.

6. A motor fuel containing gasoline and formal adapted to accelerate ignition.

7. A motor fuel containing a dialkyl ether having a boiling point below 104° C. adapted to accelerate ignition.
8. A motor fuel containing formal adapted to accelerate ignition.
9. A motor fuel containing a light hydrocarbon and less than 12% of a dialkyl ether.
10. A motor fuel having as its principal constituent, a light hydrocarbon, and a small proportion of a dialkyl ether adapted to accelerate ignition.

In testimony whereof he hereunto affixes his signature.

YASUJURO NIKAIDO.